

# UNITED STATES PATENT OFFICE.

ALFRED SCHWARZ, OF JOPLIN, MISSOURI, ASSIGNOR TO METALS RECOVERY COMPANY, OF NEW YORK, N. Y., A CORPORATION OF MAINE.

## PROCESS OF EFFECTING THE SELECTIVE FLOTATION OF MINERALS.

1,317,945.

Specification of Letters Patent.

Patented Oct. 7, 1919.

No Drawing.

Application filed June 5, 1918. Serial No. 238,280.

To all whom it may concern:

Be it known that I, ALFRED SCHWARZ, a subject of the Emperor of Germany, residing at Joplin, in the county of Jasper, State of Missouri, have invented certain new and useful Improvements in Processes of Effecting the Selective Flotation of Minerals; and I do hereby declare the following to be a full, clear, and exact description of the invention, such as will enable others skilled in the art to which it appertains to make and use the same.

This invention relates to the concentration of minerals by flotation, and more particularly to a selective method of effecting the flotation and separation of minerals.

The present invention is based upon the discovery that by the use of phenol, for example, carbolic acid, together with a small amount of a resin soap solution, it is possible to effect the selective flotation of one mineral from another, for example, lead sulfid from zinc sulfid, where the ore pulp is of an alkaline or neutral character; and that the zinc sulfid may be subsequently recovered by flotation, by a proper modification of the conditions under which the flotation is carried out.

The invention will be described more in detail in connection with the following specific instances of its application, but it will be understood that the invention will be illustrated by, but is not limited to, the specific procedures and processes thus described.

In order to effect the selective flotation of lead sulfid without separating the zinc sulfid, and thereafter effect the flotation of the zinc sulfid from the gangue, the following procedure may be followed:

A suitable lead-zinc sulfid, of the Missouri lead-zinc district, is first subjected to flotation with the addition thereto of a phenol, such as carbolic acid, and a resin soap solution. For one ton of the ore there may thus be added two pounds of carbolic acid and one-half pound of a resin soap solution containing about 2% of resin, 1% of caustic soda and 97% water. Such a resin soap solution may be made by boiling the resin, caustic soda and water for a sufficient period of time to bring the resin into solution and to give a solution which remains permanent on cooling.

The proportions of the ingredients of the

resin solution, as well as the proportions of the solution and carbolic acid or other phenol to the ore, can, of course, be varied; but the above proportions are those which I have found well adapted for effecting the desired selective flotation of the lead from the zinc.

The ore is utilized in the form of an ore pulp which will usually contain about three to five parts of water to one part of ore. The phenol and the resin solution are incorporated therewith and the ore is then subjected to a flotation treatment in any suitable type of flotation machine. I consider a pneumatic machine of the type of the Callow cell particularly adapted for the practice of the process since by its use the desired selective flotation can be readily effected. If too much agitation is used, the zinc will also tend to float and thus become mixed with the lead concentrate. If a machine of the mechanical agitation type is used, the agitation speed should be uniform and well controlled so that the zinc will not be also floated.

By proceeding in the manner above described, the lead can be obtained in the form of a concentrate and approximately complete extraction of the lead effected.

Thereafter, the ore pulp may be subjected to a further treatment for the purpose of separating the zinc from the gangue. Various methods of procedure may be followed in effecting this separation. I have, however, found it of advantage to make use of further amounts of the resin solution, and to give to the pulp an acid condition. There may thus be added to the ore pulp, after the separation of the lead, about ten pounds of the resin soap per ton of ore, and sufficient acid to establish an acid condition in the circuit water. The amount of acid may vary from, for example, 5 to 10 pounds per ton of ore, according to the particular ore used and its alkaline content. When the ore pulp is now subjected to a further flotation treatment, the zinc will be found to float and can be separated with substantial completeness from the gangue.

It will of course be understood that in practice a series of flotation machines or cells will be employed. The lead flotation may thus be made in the first machine, or in the first machines of the series, and the zinc flotation in the subsequent machines.

The intermediate machines may be employed for handling middling products in much the usual manner.

From the above specific description it will be seen that the separation of the lead is first effected by the addition of a phenol and a small amount of resin soap in an alkaline solution; and that thereafter the lead is separated by flotation after the addition 10 of further amounts of resin soap to the ore pulp and circuit water, and the addition of sufficient acid, preferably sulfuric acid, to cause the circuit water to change from an alkaline to a distinctly acid character. By 15 subjecting the ore pulp to a further flotation treatment, the zinc sulfid can be obtained in the form of the flotation concentrate and can be thus selectively separated, to a large extent, from iron sulfid present 20 in the ore. There is thus obtained a selective separation of the zinc from iron, as well as of lead from zinc, something which is highly desirable in order to obtain both lead and zinc concentrates in a condition 25 adapting them for further metallurgical treatment.

Having thus described my invention, what I claim is:

1. The method of effecting the selective 30 separation of lead and zinc sulfids from mineral pulps containing them, which comprises incorporating with the mineral pulp a small amount of a phenol and of a resin soap solution and subjecting the pulp, while non- 35 acid, to a flotation operation and thereby effecting the selective flotation of the lead sulfid, subsequently adding an acid to give to the ore pulp an acid reaction, and again subjecting the pulp to a flotation operation 40 and effecting flotation of the zinc sulfid.

2. The method of effecting the selective separation of lead and zinc sulfids from

mineral pulps containing them, which comprises incorporating with the mineral pulp a small amount of a phenol and of a resin soap 45 solution and subjecting the pulp, while non-acid, to a flotation operation, and thereby effecting the selective flotation of the lead sulfid, then adding further amounts of resin soap solution and acid and subjecting 50 the ore pulp to a further flotation operation and effecting flotation of the zinc sulfid.

3. The method of effecting the selective separation by flotation of lead and zinc sulfids from mineral pulps containing them, 55 which comprises incorporating with the mineral pulp a small amount of a phenol and of a resin soap solution, and subjecting the ore pulp, while in an alkaline condition, to a flotation operation, and thereby effecting 60 flotation of the lead sulfid, thereafter adding further amounts of resin soap solution and sufficient acid to give an acid reaction to the pulp, and subjecting the pulp to a further flotation operation and thereby effecting flotation of the zinc sulfid. 65

4. The method of effecting the selective separation of lead and zinc sulfids from mineral pulps containing them and also containing iron sulfid, which comprises incorporating with the mineral pulp a small amount of a phenol and of a resin soap solution and subjecting the pulp, while non-acid, to a flotation operation, thereby effecting 70 the selective flotation of the lead sulfid, 75 then adding further amounts of resin soap and sufficient acid to give to the ore pulp an acid reaction, and again subjecting the pulp to a flotation operation, and thereby effecting flotation of the zinc sulfid from the 80 iron sulfid.

In testimony whereof I affix my signature.

ALFRED SCHWARZ.